# EUROPEAN PATENT SPECIFICATION

(11) **EP 0 257 729 B1**
(45) Date of publication and mention of the grant of the patent: **06.02.1991**
(21) Application number: 87302855.9
(22) Date of filing: 01.04.1987
(51) Int. Cl.: B44C 1/17, B44F 11/00

(54) **Dry transfer article comprising a graphic pattern and a protective clear coat in pre-use registration therewith and method of making**
Musterungen aufweisendes Trockenübertragungsmaterial mit vor Gebrauch in Übereinstimmung gelagertem Schutzüberzug und Verfahren zu dessen Herstellung
Matériau de transfert à sec comprenant des motifs graphiques avec enduit protecteur clair superposé en registre avant usage et son mode de fabrication

(30) Priority: 01.04.1986 US 846754; 12.12.1986 US 941023
(43) Date of publication of application: 02.03.1988
(73) Proprietor: MINNESOTA MINING AND MANUFACTURING COMPANY, St. Paul, Minnesota 55133-3427 (US)
(72) Inventor: Frank, John W. c/o Minnesota Mining and, P.O. Box 33427 St. Paul Minnesota 55133 (US); Koster, Brian L. c/o Minnesota Mining and, P.O. Box 33427 St. Paul Minnesota 55133 (US); Janssen, Jeffrey R. c/o Minnesota Mining and, P.O. Box 33427 St. Paul Minnesota 55133 (US); Olson, Kenneth G. c/o Minnesota Mining and, P.O. Box 33427 St. Paul Minnesota 55133 (US)
(74) Representative: Baillie, Iain Cameron

(56) References cited:
- US-A- 3 516 842
- US-A- 4 356 617

## Description

### Field of invention

This invention relates to a thin film graphic design article, and to methods for making same. More particularly, it relates to an article comprising a thin film graphic design having a protective coating thereover, with the protective coating having tapered edges, providing an appearance which is similar to that of paint.

### Background

On site application of paint directly to a surface to be decorated is the time-honored method for providing a graphic design, such as a decorative design. While such a process provides many aesthetic and physical features, including realistic appearance, color flexibility, durability to abrasion, weathering and chemical attack, it also suffers from many disadvantages. For example, relatively skilled labor is necessary. Long application times are usually the rule, and potential contamination to adjacent areas, particularly mechanical equipment, can occur. Accordingly, prefabricated film graphics have been utilized to avoid many of these disadvantages. Such film graphics, often called "decals" or "transfer graphics", when utilized on the exterior surface of vehicles, typically require extreme resistance to abrasion and chemical attack because of exposure of the vehicle surfaces to various atmospheres or environments. Accordingly, such graphics must generally be provided with a protective clear coat over the graphic areas.

This protective clear coat can be located in registry with the graphic area by applying a continuous layer of clear coat over the graphic and non-graphic areas, and subsequently cutting through the several layers precisely at the outline of the graphic area, typically called "die cutting" or "kiss cutting". This approach results in substantially vertical or right angle edges of the graphic and protective clear coat which can collect dirt, wax, and other foreign materials which can detract from the aesthetics of the applied graphic design. Responsive thereto, a sealing agent, such as SCOTCHCAL Brand 4150 Edge Sealer, available from the Minnestoa Mining and Manufacturing Company ("3M") may be applied about the edges of such a graphic after application, e.g., to the side of a vehicle with adhesive. The sealing agent protects the exposed sides of the graphic and adhesive from chemical attack and reduces the mechanical forces acting thereon. This technique is most typically practiced in the airline industry.

A second approach is to apply the protective clear coat only to graphic areas, as, for example, by screen printing, or utilizing a stencil with an open area corresponding precisely to the outline of the graphic design. Those skilled in the art are aware of the difficulty encountered with such a process, because of factors such as dimensional changes in the film substrate, tension variables in the screen mesh, and accurate positioning of the substrate in registry with the stencil. Small graphics, such as those with overall dimensions of not greater than about 30 centimetersx30 centimeters (12 inchesx 12 inches) can generally be manufactured with satisfactory registration by those having requisite skill. However, this becomes much more difficult for larger graphic areas, and particularly for decorative items such as pin stripes which are common for the vehicle or automotive market.

U.S. Patent No. 4,356,617 (Coscia) discloses the formation of a raised dike around a graphic design for the purpose of controlling the flow of a coating composition applied thereto. The reference further teaches that such flow may also be controlled by a groove or gap around the design if the coating composition has sufficient surface tension. U.S. Patents Nos. 4,322,074 (Auld et al.) and 4,605,575 (Auld et al.) disclose utilization of integral bezels for similar purpose. Such techniques are typically not preferred because they may not provide the tapered edge which is desired of thin film graphic to impart a paint-like appearance thereto. Furthermore, the techniques disclosed in these references do not provide application of the protective clear coat to the adhesive layer which adheres the graphic design to a desired substrate, thereby leaving the edges of the adhesive exposed and subject to collection of foreign materials and environmental degradation.

Yet another approach which could be utilized is to apply the protective clear coat with a substantial oversize border to assure complete coverage of the graphic area. While this method achieves the required objective of protection for the graphic design, it is generally considered not to be aesthetic.

Although application of a protective clear coat by screen printing is a typical technique, other methods such as roller coating or spray coating may also be considered, providing a dry film thickness of from about 0.01 to 0.1 millimeters (0.5 to about 4 mils) is achieved.

Summarizing, an acceptable protective clear coat should: be of sufficient thickness to provide adequate wearability and resistance to chemical environments; precisely cover the graphic area, whether same be large or small, and whether it be a simple geometric shape, such as a narrow width line, or a complex intricate design; and provide a tapered profile to the graphic. If desired the protective clear coat should also seal the underlying adhesive which adheres the graphic to a desired substrate. Known techniques described above do not satisfy all these requirements.

Accordingly, the present invention provides precise registration of a clear protective coat over a graphic pattern; the protective coat has tapered, rounded and sloping edges which inhibit the buildup of wax and foreign matter at the edge portions, and looks integrated with the substrate; i.e., provides a paint-like look; the process kan accommodate varying process tolerances, operator variability and equipment tolerances; and the process provides a lenticular appearance on thin pin stripes, such as may be placed on vehicle surfaces. If desired, the protective coating may also cover the underlying adhesive that is used to adhere the graphic to a desired substrate, thereby sealing the edges of the adhesive to further enhance the inhibition of the buildup of wax and foreign matter at the edges of the graphic, and providing unexpected solvent resistance thereto.

### Summary of the invention

In accordance with the invention, there is a process provided for preparing a graphic pattern having a protective coating thereon in "precise registration" (as defined herein) therewith. The process comprises: 1) providing a carrier having a major surface, 2) applying, in imagewise fashion, an imaging composition on the major surface of the carrier, which composition has sufficient surface tension to wet the major surface, to provide a film of the graphic pattern thereon, 3) drying the film of graphic pattern, 4) applying a liquid protective coating over the graphic pattern, beyond the edge definition thereof and in substantial registration therewith, the protective coating composition having a surface tension sufficient to wet the graphic pattern but not the major surface of the carrier film and 5) drying the coating of protective material, whereby upon drying the protective overcoat dewets or retracts from the major surface of the carrier totally onto the graphic pattern, thus providing precise registration therewith. If desired, multicolor graphic patterns may be provided by applying, in the appropriate imagewise fashion, one or more additional layers of imaging compositions of appropriate color.

In a preferred embodiment of the invention, a dry transfer graphic article comprising a graphic pattern and underlying adhesive is provided which has a protective coating thereon in "precise registration" (as defined herein) therewith such that the graphic has rounded and sealed edges and a paint-like appearance when applied to a desired substrate. The protective clear coat covers the graphic pattern and seals the edges of the graphic pattern and also the underlying adhesive so as to protect the transfer graphic from abrasive forces and prevent collection of foreign matter at the edges of the graphic pattern and underlying adhesive. Further, the clear coat provides unexpected solvent resistance to the adhesive, thereby improving the durability and longevity of such graphics. The present invention also provides a process for making such a graphic transfer article.

Briefly summarizing, the process for making such a transfer graphic article comprises: 1) providing a carrier having a major surface; 2) coating a layer of adhesive, typically pressure-sensitive adhesive, thereon; 3) applying an imaging layer or stratum, e.g., a polymer film of desired color or layer of an imaging composition such as an ink, thereover; 4) trimming the imaging stratum and underlying adhesive in imagewise fashion to provide the desired graphic pattern, e.g., by kiss-cutting in imagewise fashion and then removing the nonimagewise portions of the same; 5) applying a liquid protective coating over the graphic pattern, beyond the edge definition thereof and in substantial registration therewith, the protective coating composition having a surface tension sufficient to wet the graphic pattern and exposed edges of the underlying adhesive, but not the major surface of the carrier; and 6) drying the coating of protective material, whereby upon drying the protective clear coat dewets or retracts from the major surface of the carrier into precise registration with the graphic pattern, sealing the edges of the graphic pattern and underlying adhesive and providing a rounded profile. If desired, one or more layers of an imaging composition, e.g., ink, may be applied to the imaging stratum to provide special effects, e.g., a multicolor graphic, etc., as discussed above.

### Brief description of drawing

The present invention is further explained with reference to the drawing which illustrates a preferred embodiment thereof wherein:
Figure 1 is a cross-sectional representation of an imaging stratum and underlying adhesive layer which have been applied to a carrier;
Figure 2 is a cross-sectional representation of the construction of Figure 1 after an image composition has been printed thereon and a desired graphic pattern has been formed by kiss-cutting and weeding in an imagewise fashion;
Figure 3 is a cross-sectional representation of the construction of Figure 2 after a liquid protective coating has been applied and dried thereon;
Figure 4 is a cross-sectional representation of the construction of Figure 3 after lamination of an application tape thereto; and
Figure 5 is a cross-sectional representation of a preferred transfer graphic of the invention being applied to a substrate.

These figures, which are not to scale, are intended to be merely illustrative and not limiting.

### Detailed description of preferred embodiment of invention

The invention relates to a process for the manufacture of a dry transfer graphic material, comprising the steps of applying an image layer, typically comprising one or more layers of ink to a substrate surface to form a graphic pattern thereon, and applying thereover, a protective clear coat, the clear coat being applied beyond the edge definition of the graphic pattern in substantial registration therewith, the surface energy of the substrate being sufficiently low relative to the surface tension of the protective clear coating that non-wetting by the protective coating occurs, and same therefor "creeps" back to the edge surface of the graphic pattern. The protective coating is thus in precise registration with the graphic pattern thereby providing an aesthetically pleasing unitary or paint-like appearance.

"Precise registration" is defined herein to mean a slight oversize border which is approximately 0.21 millimeters (5 mils) or less in width. Such borders provide the desired protection and sealing of the graphic pattern and, in some embodiments, the underlying adhesive; but are essentially undistinguishable to the unaided eye, thus clear coats having such borders appear to be in precise registration with the graphic or visually coincident therewith.

In a preferred embodiment, the invention also relates to a transfer graphic article having a protective coating thereon such that the article, including graphic pattern and underlying adhesive in registry therewith, has rounded and sealed edges. The process for the manufactur of sucy a dry transfer graphic article comprises the steps of applying to a carrier surface an imaging layer or stratum, e.g., one or more layers of an imaging composition, and underlying adhesive to form a desired graphic pattern; and applying thereover a protective clear coat, the clear coat being applied beyond the edge definition of the image areas in substantial registration therewith, the surface energy of the carrier being sufficiently low relative to the surface tension of the protective clear coating that non-wetting of the carrier by the protective coating occurs, the same therefor "creeps" back to the surface and edges of the graphic pattern and underlying adhesive into precise registration therewith.

The carrier comprises a material which inherently has a low surface energy, or has a low surface energy coating thereon, e.g., a paper or polyester film with silicone coating thereon. The carrier functions to provide a base surface having sufficient rigidity on which to coat the adhesive and apply the imaging stratum, e.g., a polymer film, and trim the same in imagewise fashion, e.g., by kiss cutting and removing weed; yet has a sufficiently low comparative surface energy such that as the clear liquid protective top coat dries thereon, same will not wet, or will retract from, the carrier surface onto the graphic film and and underlying adheive. In addition, the carrier functions as a release liner and must allow for easy release of the graphic transfer therefrom, i.e., the adhesion of the adhesive thereto should be releasable.

The imaging stratum comprises a material such as a polymer film or ink. The film is preferably a material of desired color which has a surface energy which is higher than that of the carrier such that when the protective clear coat is applied it will dewet or retract from the carrier surface onto the imaging stratum and underlying adhesive.

The underlying adhesive should provide high adhesion to the imaging stratum and desired substrate to which the ultimate graphic is applied, yet should releasably adhere to the carrier.

The adhesive may first be coated on the carrier and the imaging stratum then applied thereto, or it may first be coated on the imaging stratum, e.g., a film, following which the precoated imaging stratum is applied to the carrier. The adhesive should form a substantially continuous layer covering at least the area of the desired graphic pattern, and preferably extends at least slightly therebeyond, such that a layer of adhesive will underly substantially all of the graphic pattern, providing secure adhesion to the substrate. Examples of suitable adhesive-precoated films include SCOTCHCAL Brand 3650 Series Polyvinyl Chloride Films, and SCOTCHAL Brand 5690 Series Polyester Films, which have acrylic type pressure-sensitive adhesives on the back side and are available from the Minnesota Mining and Manufacturing Company ("3M").

Figure 1 shows carrier 10 comprising a polymer film 12 with surface 14 having a low surface energy to which adhesive 16 and imaging stratum 18 have been applied.

If desired, e.g., for multi-color graphic patterns, one or more layers of imaging compositions or materials may be coated or printed on the imaging stratum in desired pattern.

The imaging material can be comprised of conventional imaging materials used to form graphic images on substrates, such as inks, for example. The exact composition of the imaging material depends on the end use properties required. The imaging material is typically applied from a wet composition having surface tension properties such that the composition will wet out and flow on the imaging straum to form a film and provide a visible printed pattern thereon. Imaging materials may be colored or colorless, although colored compositions are preferred. If desired, special effects may be achieved if the composition provides a product which is visible under ultraviolet light, but is colorless under ordinary ambient light. Conventional inks can be utilized, such as the vinyl or vinyl acrylic inks whihc are commercially available.

Screen printable inks can be classified on the basis of formation of an ink film, and the vehicles used for that film formation. For examples, solvent-based inks form a film by evaporation of the various solvents contained therein, i.e., the wet film is dried. Curable inks provide a film which becomes polymerized through chemical change. Examples of inks include enamels; solvent-based inks, e.g., those containing lacquers and other solvents, poster inks, and water-based inks; those containing 100 percent solids, such as those based on epoxies, ultraviolet exposure systems, plastisols, etc.; and specialty inks, such as those which are expandable, those which exhibit electrical properties, etc.

To obtain good wetting, i.e., maximum surface contact on the imaging stratum, and the surface tension of the ink must be equal to or less than the critical surface tension of the imaging stratum. In other words, the imaging stratum must have a higher degree of surface wetability than the imaging composition. However, the surface tension of the film formed by the imaging composition must be greater than that of the carrier surface such that the protective coating will properly dewet from the carrier surface to achieve desired registration with the graphic. If the surface tension of the film formed by the imaging composition is not sufficiently greater than that of the carrier surface, precise registration of the clear coat with the graphic pattern may not be achieved. Specific solvents, surfactants, and other conventional and known additives can be utilized to modify the surface properties of the imaging composition, as desired.

Multiple imaging composition films, such as of different colors, may also be printed in sequence if desired.

The imaging stratum, imaging composition film, if any, and underlying adhesive are then trimmed in an imagewise fashion to provide the desired graphic pattern, such as by kiss cutting in imagewise fashion and removing undesired portions, i.e., weed. Care should be taken when kiss cutting because cutting too deeply, i.e., into the carrier, may tend to cause the clear coat composition to incompletely dewet from the carrier during drying, thus causing the final clear coat to only partially seal the edges of the graphic pattern and adhesive, whereas failure to cut deeply enough, i.e., not completely through the adhesive layer, may interfere with complete stripping of the weed. Figure 2 shows adhesive 16, imaging stratum 18, and imaging composition film 20 on carrier 10 after kiss-cutting and weeding to form the desired graphic pattern.

This invention relates to a process utilizing the surface tension characteristics of each of the four components of the process, i.e., the carrier surface, the imaging stratum, and imaging composition, if any, and the protective clear coat. Usually, one begins with a determination of the critical solid surface tension of the carrier surface and then tailors the other components to meet the requisite surface tension requirements. The surface energy of a film can be determined in a number of ways. For example, a series of liquids of known surface tension can be applied to a smooth test surface. The contact angle of these liquids on the solid surface is measured, and this information can then be plotted against the known surface tension of the respective liquids. Extrapolation of such data to a zero contact angle provides the solid surface tension, i.e., that of the carrier surface, since at this point the surface tension of the solid film is approximately equal to that of the liquid. This surface tension thus becomes the critical solid surface tension. When utilizing this procedure with a silicone-coated carrier, surface tension was calculated to be 23.8 dynes/centimeter, which is in agreement with the reported literature value of 24 dynes/centimeter.

Similarly, results of contact angle measurements for liquids having known values of liquid surface tension due to dispersion forces and polar forces, both of which contribute to surface free energy can be utilized.

Finally, wetting tension test kits are commercially available to determine the critical surface tension of specific film substrates.

Examples of typical surface tension values include about 32 dynes/centimeter for polyvinyl chloride films which can typically be corona treated to yield values of about 60 to 70 dynes/centimer, and about 26 to 35 dynes/centimeter for typical vinyl inks which can also be corona treated to yield surface energies of greater than 60 dynes/centimeter.

Once the critical solid surface energy of the carrier surface is known, an imaging stratum can be selected and an imaging composition can be tailored thereto to provide or produce a good graphic pattern which can be clear coated with the desired precise or visually coincident registration.

Once the desired graphic pattern is appropriately formed on the carrier surface, the protective clear coat can be formulated based on solvent selection, particular resin, and other additives which together provide a formulation which is capable of wetting the dry graphic pattern and exposed adhesive layer sufficiently, and yet is not capable of wetting the carrier surface.

Other critical factors include the solvation of the coating composition and its rate of drying, in addition to its relative surface tension.

The protective clear coat is made typically of a resinous film-forming material, an example thereof being aliphatic polyurethanes, which are conventionally utilized today to provide a protective top coat for a transfer graphic image.

The liquid top coat is printed, as by screen printing, for example, over the grahic pattern, and slightly beyond the edge definition thereof, i.e., typically with an overprint margin up to about 2.54 millimeters (100 mils) wide, so as to assure complete coverage of the graphic pattern. As this liquid coat dries, it will dewet, i.e., creep or retract from the carrier where it has been overprinted onto the graphic pattern into precise registration therewith, and can be cured in conventional fashion. Preferably, the liquid is printed at least 0.12 millimeter (5 mils) beyond the edge of the graphic pattern to ensure complete sealing of the edges of same and underlying adhesive. Overprint margins of increasing width may cause the overcoat to puddle on the carrier or to bridge gaps within the graphic pattern, e.g., spaces between parallel strips such as are provided for "racing" stripes used for automotive decoration.

Accordingly, the protective clear coat provides a variable high thickness over the surface of the graphic pattern and seals the edges of the graphic pattern and underlying adhesive. Thus the clear coat protects the graphic pattern and underlying adhesive from chemical and environmental attack, thereby increasing the durability thereof, and also provides a unitary, paint-like appearance, thereby improving the attractiveness thereof.

Preferably the final thickness of the clear coat is at least 0.01 millimeter (0.5 mil), and not greater than about 0.1 millimeter (4 mils). Thinner clear coats tend to provide less effective protection to the graphic pattern and underlying adhesive whereas those substantially thicker than the indicated range may tend to give the graphic an undesirable artificial appearance.

Figure 3 shows the rounded profile provided by clear coat 22 after it has dried. The edges 24 of imaging stratum 18, underlying adhesive 16, and imaging composition film 20 have been sealed by clear coat 22.

Surprisingly, in addition to preventing collection of foreign matter at the edges of the transfer article, it has been found that the clear coat provides excellent solvent resistance to the graphic, particularly to the underlying adhesive. Thus it is preferred that the clear coat and underlying adhesive are mutually reactive to achieve an optimum seal. For instance, an isocyanate-containing clear coat composition and acrylic acid- containing adhesive will typically react to provide a chemical bond between the adhesive layer and clear coat, such a bond typically providing exceptional solvent resistance to the adhesive layer.

As shown in Figure 4, the article can then be laminated to a conventional application tape 26, i.e., a flexible film 28 having a low-tack adhesive 30 thereon, whereupon imaging composition film 20, imaging stratum 18, underlying adhesive 16, and overlying protective coat 22 can be stripped away from the carrier 10, which can then be discarded, and the transfer article then applied to a substrate. Following burnishing action, e.g., with a squeegee, the application tape is removed leaving the transfer article adhered to the substrate. Figure 5 shows the transfer article adhered to substrate 32 after application tape 26 has been partially removed.

In this manner, there is provided a low profile, high performance, durable graphic transfer system, having special utility in the automotive market place. For example, the invention can provide an automotive stripe or marking which is unique in appearance and performance properties, in that the graphics produced by the invention have rounded edges and closely similate paint, a technique not heretofor available with a transfer graphic system. Further, the graphics disclosed herein are very durable and resistant to force typically encountered by automobile finishes, e.g., abrasive action, dirt impact, and solvent attack.

The invention will now be further illustrated by the following illustrative examples, wherein all parts are by weight unless otherwise specified.

### Example 1

A SCOTCHCAL Brand 3655 Film comprising a polyvinyl chloride film coated with an acrylic pressure-sensitive adhesive protected with a silicone coated paper release liner was used as the imaging stratum, underlying adhesive, and carrier.

The film and underlying adhesive were hot kiss cut in an imagewise fashion ("racing" stripes) using a Teflon-coated, etched magnesium die at a temperature of 175°C (350°F) to produce edges with a tapered profile.

The weed was then removed from the carrier to produce the graphic pattern.

A clear coat was then applied to the graphic pattern with an overprint margin of about 0.50 to 1.0 millimeter (20 to 40 mils) using a 110 mesh screen. The clear coat, a two component polyurethane, had the following formulation:

The clear coat was cured at 75°C (165°F) for one hour.

An application tape was laminated to the transfer graphic article.

The graphic was applied to a painted steel plate substrate.

The transfer graphic had rounded, unitary appearance similar to that of paint.

The solvent resistance of the graphic was tested by soaking the graphic and substrate in a solution comprising 90 parts unleaded gasoline and 10 parts ethanol for about 40 minutes at room temperature. After being removed, the dried transfer graphic retained its initial, paint-like appearance, having suffered no apparent degradation.

### Example 2

A transfer graphic was made and applied to a substrate as in Example 1.

Solvent resistance was tested by soaking the graphic and substrate in toluene for about 5 minutes at room temperature. After being removed and dried, the transfer graphic retained its initial, paint-like appearance, having suffered no apparent degradation.

### Example 3

A transfer graphic article was made as in Example 1, except the clear coat was a lacquer acrylic based material having the following formulation:

After application to a painted steel substrate, the transfer graphic also had a rounded, unitary appearance similar to that of paint.

### Example 4

A transfer graphic article was made as in Example 1, except the clear coat was an ultraviolet curable material having the following formulation:

The clear coat was applied to the graphic pattern with an overprint margin of about 5 to 125 mils (0.12 to 3.18 millimeters) using a 110 mesh screen.

The clear coat was cured by actinic radiation in a Linde PS-121 Photocure chamber at a beltspeed of 30 feet (9.1 meters) per minute in a nitrogen atmosphere.

After application to a painted steel substrate, the transfer graphic also had a rounded, unitary appearance simklar to that of paint.

### Example 5

A transfer graphic article was made as in Example 1, except an ink was screen printed onto the imaging stratum prior to kiss-cutting. The ink was SCOTCHCAL Brand 3905 Ink, a polyvinyl chloride/vinyl acetate copolymer-based ink pigmented with carbon black. The ink was screen printed with a 230 mesh screen and cured at 90°C (190°F) for 3 minutes.

After cooling to room temperature, a clear coat was applied thereto as in Example 1.

Following application to a painted steel substrate as in Example 1, the transfer graphic had a rounded, unitary appearance similar to two parallel stripes of paint, e.g., "racing" stripes.

### Example 6

A polyester film was coated with the following silicone composition:

(The foregoing all being commercially available from the General Electric Company).

An ink compositon was then screen printed on the silicone-coated polyester with a 110 mesh screen, the composition of the ink being:

diluted with diisoamyl ketone to provide a viscosity of 1300 cps (using a Brookfield viscometer No. 3 spindle). After printing, the solvents were evaporated by heating in an air convection oven at 75°C (165°F).

A protective clear coat having the same formulation as that used in Example 1 was diluted with CARBITOL ACETATE to a viscosity of 500 cps (using a Brookfield visometer, No. 3 spindle).

This formulation was then screen printed over the previously prepared ink image with an overprint margin of about 0.50 millimeter (20 mils).

The construction was then baked for two hours at about 75°C (165°F). During drying, the coating composition dewetted back to the edges of the ink image, thus providing excellent registration with the underlying ink areas and an attractive, paint-like appearance.

An application tape, 25-508-LC, available from Laminated and Coated Products, Inc., comprising a 0.06 millimeter (2.5 mil) polyethylene backing coated with a low-tack, water-based acrylic pressure-sensitive adhesive, was laminated to the polyester film over the coated graphic pattern. The polyester film was removed, transferring the graphic pattern from the polyester film to the application tape.

The underside of the graphic pattern and exposed portions of the low-tack adhesive on the application tape were corona treated using 500 Watts at a speed of 6.1 meters (20 feet) per minute.

An adhesive formulation, comprising 19.6 weight percent adhesive polymer (isooctyl acrylate/vinyl acetate/acrylic acid in a 74/22/4 weight ratio) and 80.4 weight percent ethyl acetate, was prepared by mixing the ingredients together at room temperature; coating the solution onto a silicone-coated, white polyethylene film 05-5-HiD-ST6A/ST3A-White available from Schoeller Release Products, Inc., to a wet thickness of about 0.8 millimeter (3 mils); and evaporating the solvent by heating for five minutes at 75°C (165°F). The adhesive-coated side of this film was laminated to the corona-treated side of the application tape and graphic pattern.

The silicone-coated polyethylene film was removed and the article placed on a painted steel substrate such that adhesive was in contact with the painted steel. Moderate pressure was applied to the application tape by stroking that surface with the edge of a polyethylene squeegee over the film structure. The application tape was then peeled from the substrate. The graphic design remained on the painted steel substrate and any adhesive not in registration with the graphic article remained on the application tape.

The solvent resistance of the article was then tested by immersion in a gasoline/ethanol mixture as in Example 1. After removal and drying, the graphic article was inspected to reveal disfiguring solvent attack along the edges thereof. The ink image had become rippled and rough along the edges thereof and the underlying adhesive in such areas had been leached out.

### Comparative Example A

A continuous layer of the protective clear coat composition described in Example 1 was applied to SCOTCHCAL Brand 3655 Film by screen printing the composition through a 110 mesh screen. The clear coat was cured at 75°C (165°F) for one hour.

The clear coat, film, and underlying adhesive were hot kiss-cut in an imagewuse fashion ("racing" stripes) using a Teflon-coated, etched magnesium die at a temperature of 175°C (350°F).

The weed was then removed from the carrier to produce a graphic article. The edges of the article did not have a rounded profile such as would suggest a paint-like appearance.

An application tape was laminated to the graphic article, and the article was applied to a painted steel substrate as in Example 1.

The solvent resistance of the graphic was then tested by immersion in a gasoline/ethanol mixture as in Examples 1 and 6. After removal and drying, the graphic was inspected whereupon it was observed that the adhesive had oozed from underneath the graphic pattern.

In each of Examples 1-6, all examples of the invention, the graphic articles produced had rounded profiles and a paint-like appearance. Comparison of the results of Examples 1 and 2, preferred embodiments of the invention, with those of Example 6 and Comparative Example A illustrates the solvent resistance achieved by a preferred transfer graphic of the invention wherein the protective clear coat seals both the graphic pattern and underlying adhesive and the improved solvent resistance attained as compared to that of transfer graphics wherein the clear coat is applied only to the graphic pattern and not to be exposed edges of the underlying adhesive.

Various modifications and alterations of this invention will become apparent to those skilled in the art without departing from the scope of the claims of this invention.

## Claims

1. A dry transfer article for application to a substrate to provide a design thereon, characterized in that said article comprises:
A) a graphic pattern (18);
B) a layer of adhesive (16) underlying said graphic pattern (18) in exact registration therewith; wherein said adhesive is capable of providing adhesion to said graphic pattern and said substrate; and
C) a protective clear coat (22) in precise registration with said graphic pattern (18) and said layer of adhesive (16), said clear coat having a rounded profile, covering said graphic pattern, and sealing the edges (24) of said graphic pattern and said adhesive layer.

2. The article of Claim 1 further characterized in that said graphic pattern comprises a film.

3. The article of Claim 2 further characterized in that said graphic pattern further comprises a film of at least one imaging composition which covers at least a portion of the surface of said graphic pattern.

4. The article of any one of Claims 1-3 further characterized in that said protective clear coat comprises an aliphatic polyurethane.

5. The article of any one of Claims 1-4 further characterized in that said protective clear coat is curable with ultraviolet radiation.

6. The article of any one of Claims 1-5 further characterized in that said protective clear coat has reacted with said adhesive.

7. The article of Claim 6 further characterized in that said protective clear coat contains an isocyanate and said adhesive contains acrylic acid.

8. The article of any of Claims 1-7 further characterized in that said article comprises a release liner.

9. The article of Claim 8 further characterized in that said article comprises an application tape.

10. A process for preparing a graphic pattern on a substrate, the graphic pattern having a protective coating (22) thereover and in exact registration therewith, characterized in that said process comprises:
A) providing a carrier film (10) having a major surface thereon;
B) applying at least one coating of an imaging composition (18) on said major surface, said imaging composition having a sufficient surface tension to wet said major surface of said carrier and provide a film of said graphic pattern thereon;
C) drying said coating of imaging composition (18) to form said graphic pattern;
D) applying a liquid protective coating (22) over said graphic pattern, beyond the edge definition (24) thereof and in substantial registration therewith; said protective coating having sufficient surface tension to wet said graphic pattern, but not said major surface of said carrier film (10);
E) drying said liquid protective coating (22); whereby during said drying said protective coating (22) will dewet and retract from said major surface of said carrier onto said graphic pattern and provide exact registration with said graphic pattern.

11. A process for preparing a dry transfer article capable of transfer of a graphic pattern to a substrate, said graphic pattern having a protective coating (22) thereover in precise registration therewith which seals underlying adhesive (16), charactzrized in that said process comprises:
A) providing a carrier (10) having a major surface thereon;
B) coating an adhesive layer (16) thereon;
C) applying an imaging stratum (18) thereover;
D) trimming said imaging stratum and underlying adhesive in an imageweise fashion to provide a graphic pattern;
E) applying a liquid protective coating (22) over said graphic pattern, beyond the edge definition (24) thereof and in substantial registration therewith; said protective coating having sufficient surface tension to wet said graphic pattern and exposed adhesive, but not said major surface of said carrier (10); and
F) drying said protective coating (22); whereby during said drying said protective coating will dewet and retract from said major surface of said carrier and provide precise registration with said graphic pattern, sealing the edges of same and said underlying adhesive.

12. The process of any one of Claims 10 or 11 further characterized in that said carrier film is a polyester.

13. The process of any one of Claims 10 or 11 further characterized in that said major surface has a low surface energy coating thereon.

14. The process of Claim 13 further characterized in that said low surface energy coating is a silicone.

15. The process of Claim 11 further characterized in that at least one layer of an imaging composition is applied to said imaging stratum in imagewise fashion.

16. The process of any one of Claims 10 or 15 further characterized in that said imaging composition comprises an ink.

17. The process of Claim 16 further characterized in that said ink is selected from the group consisting of vinyl and vinyl-acrylic inks.

18. The process of any one of Claims 10 or 11 further characterized in that said protective coating composition comprises an aliphatic polyurethane.

19. The process of any one of Claims 10 or 11 further characterized in that said protective coating composition is curable with ultraviolet radiation.

20. The process of any one of Claims 10 or 11 further characterized in that said process comprises the steps of curing said protective coating after the drying thereof.

21. The process of Claim 11 further characterized in that said protective overcoating is reactive with said adhesive.

22. The process of Claim 21 further characterized in that said liquid protective coating comprises an isocyanate and said adhesive layer comprises acrylic acid.

## Patentansprüche

1. Trockenumdruckartikel zum Auftragen auf ein Substrat, um dieses mit einem Muster zu versehen, dadurch gekennzeichnet, daß der Artikel besitzt:
A) ein graphisches Muster (18);
B) eine Klebstoffschicht (16) unter dem graphischen Muster (18) mit ihm genau korrespondierend angeordnet, so daß der Klebstoff zum Kleben an dem graphischen Muster und dem Susbtrat befähigt ist; und
C) einem mit dem graphischem Muster (18) und der Klebstoffschicht (16) genau korrespondierenden, klaren Schutzüberzug (22), der ein abgerundetes Profil hat, das graphische Muster bedeckt und die Ränder (24) des graphischen Musters und der Klebstoffschicht versiegelt.

2. Artikel nach Anspruch 1, dadurch gekennzeichnet, daß das graphische Muster eine Folie aufweist.

3. Artikel nach Anspruch 2, dadurch gekennzeichnet, daß das graphische Muster ferner eine aus mindestens einer Bilddarstellungszusammensetzung bestehende Schicht aufweist, die wenigstens einen Teil der Oberfläche des graphischen Musters bedeckt.

4. Artikel nach einem der Ansprüche 1 bis 3, dadurch gekennzeichnet, daß der klare Schutzüberzug wenigstens teilweise aus einem aliphatischen Polyurethan besteht.

5. Artikel nach einem der Ansprüche 1 bis 4, dadurch gekennzeichnet, daß der klare Schutzüberzug durch Ultraviolettstrahlung härtbar ist.

6. Artikel nach einem der Ansprüche 1 bis 5, dadurch gekennzeichnet, daß der klare Schutzüberzug mit dem Klebstoff reagiert hat.

7. Artikel nach Anspruch 6, dadurch gekennzeichnet, daß der klare Schutzüberzug ein Isocyanat enthält und daß der Klebstoff Acrylsäure enthält.

8. Artikel nach einem der Ansprüche 1 bis 7, dadurch gekennzeichnet, daß der Artikel eine Antihaftauflage besitzt.

9. Artikel nach Anspruch 8, dadurch gekennzeichnet, daß der Artikel ein Anbringband besitzt.

10. Verfahren zum Herstellen eines graphischen Musters auf einem Substrat, wobei das graphische Muster oben mit einem mit dem Muster genau korrespondierenden Schutzüberzug (22) versehen ist, dadurch gekennzeichnet, daß in dem Verfahren:
A) eine Trägerfolie (10) mit einer obenliegenden Breitseitenfläche verwendet wird;
B) auf die genannte Breitseitenfläche mindestens ein Überzug aus einer Bilddarstellungszusammensetzung (18) aufgetragen wird, die eine solche Oberflächenspannung besitzt, daß die Zusammensetzung die genannte Breitseitenfläche des Trägers benetzt und darauf eine Schicht aus dem graphischen Muster bildet;
C) durch Trocknen des Überzuges aus der Bilddarstellungszusammensetzung (18) das graphische Muster gebildet wird;
D) auf das graphische Muster über seine Randbegrenzung (24) hinaus eine mit dem Muster im wesentlichen korrespondierende Schutzüberzugsflüssigkeit (22) aufgetragen wird, die eine solche Oberflächenspannung besitzt, daß die Flüssigkeit das graphische Muster, aber nicht die genannte Breitseitenfläche der Trägerfolie (10) benetzt;
E) die Schutzübetzugsflüssigkeit (22) getrocknet wird, so daß während dieses Trocknens der Schutzüberzug von der genannten Breitseitenfläche des Trägers entnetzt wird und sich von dieser Fläche auf das graphische Muster in genauer Korrespondenz mit diesem zurückzieht.

11. Verfahren zum Herstellen eines Trockenumdruckgegenstandes für den Umdruck eines graphischen Musters auf ein Substrat, wobei das graphische Muster oben mit einem mit dem Muster genau korrespondierenden Schutzüberzug (22) versehen ist, der einen darunter befindlichen Klebstoff (16) versiegelt, dadurch gekennzeichnet, daß das Verfahren umfaßt:
A) es wird ein Träger (10) mit einer Breitseitenfläche verwendet;
B) darauf wird eine Klebstoffschicht (16) aufgetragen;
C) darauf wird eine Bilddarstellungsschicht (18) aufgetragen;
D) durch bildmäßiges Zuschneiden der Bilddarstellungsschicht und des darunter befindlichen Klebstoffes wird ein graphisches Muster hergestellt;
E) auf das graphische Muster und über dessen Randbegrenzung (24) hinaus wird mit dem Muster im wesentlichen korrespondierend eine Schutzüberzugsflüssigkeit (22) aufgetragen, die eine solche Oberflächenspannung hat, daß die Flüssigkeit das graphische Muster und den freiliegenden Klebstoff, aber nicht die genannte Breitseitenfläche des Trägers (10) benetzt; und
F) der Schutzüberzug (22) wird getrocknet, so daß während dieses Trocknens der Schutzüberzug von der genannten Breitseitenfläche des Trägers entnetzt wird und sich von dieser Fläche auf das grapische Muster in genaeur Korrespondenz mit diesem zurückzieht und dessen Ränder und der darunter befindlichen Klebstoff versiegelt.

12. Verfharen nach Anspruch 10 oder 11, dadurch gekennzeichnet, daß die Trägerfolie ein Polyester ist.

13. Verfahren nach Anspruch 10 oder 11, dadurch gekennzeichnet, daß auf der genannten Breitseitenfläche ein Überzug mit geringer Oberflächenenergie vorgesehen ist.

14. Verfahren nach Anspruch 13, dadurch gekennzeichnet, daß der Überzug mit geringer Oberflächenenergie aus einem Silicon besteht.

15. Verfahren nach Anspruch 11, dadurch gekennzeichnet, daß auf die Bilddarstellungsschicht mindestens eine Schicht aus einer Bilddarstellungszusammensetzung bildmäßig aufgetranen wird.

16. Verfahren nach Anspruch 10 oder 15, dadurch gekennzeichnet, daß die Bilddarstellungszusammensetzung wenigstens teilweise aus einer Farbzusammensetzung besteht.

17. Verfahren nach Anspruch 16, dadurch gekennzeichnet, daß die Farbzusammensetzung aus der Gruppe ausgewählt ist, die aus den Farbzusammensetzungen auf Vinyl- und Vinyl-Acrylbasis besteht.

18. Verfahren nach Anspruch 10 oder 11, dadurch gekennzeichnet, daß die Schutzüberzugszusammensetzung wenigstens teilweise aus einem aliphatischen Polyurethan besteht.

19. Verfahren nach Anspruch 10 oder 11, dadurch gekennzeichnet, daß die Schutzüberzugszusammensetzung durch Ultraviolettstrahlung härtbar ist.

20. Verfahren nach Anspruch 10 oder 11, dadurch gekennzeichnet, daß in dem Verfahren der Schutzüberzug nach seinem Trocknen gehärtet wird.

21. Verfahren nach Anspruch 11, dadurch gekennzeichnet, daß der Schützüber zur Reaktion mit dem Klebstoff fähig ist.

22. Verfahren nach Anspruch 21, dadurch gekennzeichnet, daß die Schutzüberzugsflüssigkeit wenigstens teilweise aus einem Isocyanat besteht und daß die Klebstoffschicht wenigtens teilweise aus Acrylsäure besteht.

## Revendications

1. Article de transfert à sec destiné à être appliqué à un substrat pour y former un dessin, caractérisé en ce qu'il comprend:
A) une représentation graphique (18);
B) une couche d'adhésif (16) en dessous de cette représentation graphique (18) en correspondance exacte avec cette dernière, cet adhésif étant capable d'assurer un adhérence à cette représentation graphique et au substrat susdit;
C) un revêtement transparent protecteur (22) en correspondance précise avec la représentation graphique susdite (18) et la couche précitée d'adhésif (16), ce revêtement transparent présentant un profil arrondi, en recouvrant la représentation graphique précitée, et en scellant les bords (24) de cette représentation graphique et de cette couche d'adhésif.

2. Article suivant la revendication 1, caractérisé en outre en ce que la représentation graphique susdite consiste un un film.

3. Article suivant la revendication 2, caractérisé en outre en ce que la représentation graphique susdite comprend en outre un film d'au moins une composition de formation d'image, qui recouvre au moins une partie de la surface de la représentation graphique précitée.

4. Article suivant l'une quelconque des revendications 1 à 3, caractérisé en outre en ce que le revêtement transparent protecteur précité consiste en un ployuréthanne aliphatique.

5. Article suivant l'une quelconque des revendications 1 à 4, caractérisé en outre en ce que le revêtement transparent protecteur est durcissable par rayonnement ultraviolet.

6. Article suivant l'une quelkonque des revendications 1 à 5, caractérisé en outre en ce que le revêtement transparent protecteur réagit avec l'adhésif.

7. Article suivant la revendication 6, caractérisé en outre en ce que le revêtement transparent protecteur contient un isocyanate, et l'adhésif contient de l'acide acrylique.

8. Article suivant l'une quelconque des revendications 1 à 7, caractérisé en outre en ce qu'il comprend une garniture de séparation.

9. Article suivant la revendication 8, caractérisé en outre en ce qu'il comporte une bande d'application.

10. Procédé de préparation d'une représentation graphique sur un substrat, cette représentation graphique comportant, par-dessus, un revêtement protecteur (22) en correspondance exacte avec elle, ce procédé étant caractérisé en ce qu'il comprend:
A) l'utilisation d'un film de support (10) présentant une surface principale;
B) l'application d'au moins une couche d'une composition de formation d'image (18) sur la surface principale susdite, cette composition de formation d'image ayant une tension superficielle suffisante pour humidifier la surface principale précitée du support et pour y former un film de la représentation graphique;
C) le séchage de la couche de compression de formation d'image (18) pour réaliser la représentation graphique précitée;
D) application d'un revêtement protecteur liquide (22) par-dessus la représentation graphique jusqu'au-delà des bords (24) de cette dernière et en correspondance pratique avec elle ce revêtement protecteur ayant une tension superficielle suffisante pour humidifier la représentation graphique mais non pas la surface principale du film de support susdit (10);
E) le séchage du revêtement protecteur liquide (22) de sorte que, durant ce séchage, le revêtement protecteur (22) se déshumidifiera et se rétractera depuis la surface principale du support sur la représentation graphique, en assurant une correspondance exact avec cette représentation graphique.

11. Procédé de préparation d'un article de transfert à sec, pouvant transférer une représentation graphique sur un substrat, cette représentation graphique comportant un revêtement protecteur (22) qui est en correspondance précise avec elle et qui scelle un adhésif sous-jacent (16), caractérisé en ce qu'il comprend:
A) l'utilisation d'un support (10) présentant un surface principale;
B) l'application d'un couche d'adhésif (16) sur ce support;
C) l'application d'un stratum de formation d'image (18) par-dessus;
D) le découpage de ce stratum de formation d'image et de l'adhésif sous-jacent d'une manière propre à former une image pour donner une représentation graphique;
E) l'application d'un revêtement protecteur liquide (22) par dessus la représentation graphique, au-delà des bords (24) de celle-ci et en correspondance pratique avec elle, le revêtement protecteur susdit présentant une tension superficielle suffisante pour humidifier la représentation graphuque et l'adhésif exposé mais par la surface principale susdite du support (10); et
F) le séchage du revêtement protecteur (22), de sorte que, durant ce séchage, le revêtement protecteur se déshumidifiera et se rétractera depuis la surface principale susdite du support et se placera en correspondance précise avec la représentation graphique susdite en scellant les bords de celle-ci et de l'adhésif sous-jacent.

12. Procédé suivant l'une ou l'autre des revendications 10 et 11, caractérisé en outre en ce que le film de support susdit est constitué par un polyester.

13. Procédé suivant l'une ou l'autre des revendications 10 et 11, caractérisé en outre en ce que la surface principale précitée comporte un revêtement de faible énergie superficielle.

14. Procédé suivant la revendication 13, caractérisé en outre en ce que le revêtement à faible énergie superficielle est constitué par une silicone.

15. Procédé suivant la revendication 11, caractérisé en outre en ce qu'au moins une couche d'une composition de formation d'image est appliquée au stratum de formation d'image de manière propre à former une image.

16. Procédé suivant l'une ou l'autre des revendications 10 et 15, caractérisé en ce que la composition de formation d'image comprent une encre.

17. Procédé suivant la revendication 16, caractérisé en outre en ce que l'encre susdite est choisie dans le groupe comprenant les encres vinyliques et les encres vinyl acryliques.

18. Procédé suivant l'une ou l'autre des revendications 10 et 11, caractérisé en outre en ce que la composition de revêtement protecteur comprend un polyuréthane aliphatique.

19. Procédé suivant l'une ou l'autre des revendications 10 et 11, caractérisé en outre en ce que la composition de revêtement protecteur est durcissable sous un rayonnement ultraviolet.

20. Procédé suivant l'une ou l'autre des revendications 10 et 11, caractérisé en outre en ce qu'il comprend la phase du durcissement du revêtement protecteur après son séchage.

21. Procédé suivant la revendication 11, caractérisé en outre en ce que le recouvrement protecteur est réactif avec l'adhésif précité.

22. Procédé suivant la revendication 21, caractérisé en outre en ce que le revêtement protecteur liquide comprend un isocyanate, et le couche susdite s'adhésif comprend de l'acide acrylique.
